

# UNITED STATES PATENT OFFICE.

HAROLD F. WHEELOCK, OF DENVER, COLORADO, ASSIGNOR TO THE SWAN PROCESS OIL COMPANY, OF DENVER, COLORADO, A CORPORATION OF COLORADO.

## UNCTUOUS COMPOSITION OF MATTER FOR MECHANICAL USAGES.

1,362,161.

Specification of Letters Patent. Patented Dec. 14, 1920.

No Drawing.

Application filed April 7, 1919. Serial No. 287,996.

To all whom it may concern:

Be it known that I, HAROLD F. WHEELOCK, a citizen of the United States, residing at the city and county of Denver and State of 5 Colorado, have invented a new and useful Unctuous Composition of Matter for Mechanical Usages, of which the following is a specification.

This invention relates to an unctuous composition of matter for mechanical usages, and more particularly embodies a more or 10 less greasy admixture of an absorptive silicious base, reduced by a fluid or semifluid lubricant to a pasty consistency, rendering 15 it peculiarly effective for certain applications as hereinafter specified.

The primary object of the invention is the production of such a thickened or salve-like compound to be applied between 20 acting bearing surfaces of certain mechanically associated parts, such as brake-drums and their coöperating brake-bands, serving as a sound-deadening or anti-squeak compound, but without sufficient antifriction 25 lubricating properties as to promote a slipping or non-gripping action, and hence ineffective binding, between the braking elements, when braking is desired.

As applied to braking elements, straight 30 oils and other true lubricants are manifestly inadequate, both because they too fully lubricate the parts, resulting in absolute slipping, an obviously serious objection, and also because, owing to their mobile nature, 35 they run off too freely to waste, and the parts soon become dry and squeaky again. The ordinary oily plastic substances or greases meet with the same objections, the overcoming of which has been attempted by 40 the use of soap-like wafers and analogous substances, but likewise they have proven to be inadequately substantial, more especially in that they are susceptible to rapid deterioration and wearing away, and a satisfactory base must be employed which will 45 absorbingly retain, in a plastic state, its impregnating lubricant the greatest length of time.

It is essentially desirable, therefore, that 50 such compounds primarily have maximum cohesiveness, in avoidance of decomposition, with a minimum slippery property, but of slightly adhesive tenacity, to just sufficiently grease or ease up the braking elements with-

out impairing their effective binding by a 55 freer lubrication thereof—thus insuring safety first at all events; and secondarily that they be not only of a more or less pasty or salve-like immobility, but also that the admixture has the important characteristics of not being easily worn out by mechanical wear nor liable to become unduly gummy, thus insuring an almost indefinitely prolonged effective use without a renewed 60 application. 65

It is now well understood that lubricating oils do not wear out mechanically, and I have discovered that an absorptive silicious base, generically, therefor proves very effective; but that even better results are assured by the use of infusorial silica, and more particularly ground-up uncalcined kieselguhr, which when admixed with a lubricating oil of low viscosity provides a 70 spongy mass of approximately correct characteristics. 75

The kieselguhr may be used in its natural 80 mined state, after pulverization, it being readily reducible to a powder as soft and smooth as a milled flour; but in actual practice I find that I may very satisfactorily utilize the filtration cakes formed in carrying out certain oil purifying processes, employing inert powdered kieselguhr as an absorptive and flotative filtering medium, 85 both in point of economy, by reclaiming an otherwise waste residue, and also because such filtration waste matter, when properly treated, functions in my improved compound with pronounced beneficial results 90 even over the use of uncalcined or raw kieselguhr. The "certain oil purifying processes" mentioned may be specifically identified by reference to the O. C. Swan United States Letters Patent issued on December 18, 1917, under #1,250,526 and 95 #1,250,527.

These oil filtration cakes, especially when removed from such purification systems, as aforesaid, for reclaiming used lubricating 100 oils from automobile engines, naturally retain a small amount of oil, not expressed therethrough, together with certain absorbed foreign substances such as road dust probably, worn away or ground up metal, 105 suspended carbon, and doubtless some colloidal or other organic matter from the oils treated, which combination, for reasons not

immediately explainable, appears to afford a more tenaciously substantial body than does even raw kieselguhr for my particular purposes; but at any event the resultant 5 filtration cake is in the nature of a semi-dry sponge-like substance peculiarly adapted for the improved admixture when ground up into a pulpous mass.

As a specific example of a proper quantity of each ingredient, when plain or free 10 kieselguhr or the like is used, the composition may be thoroughly admixed in approximately the following proportions:

Crushed kieselguhr ----- 12 pounds.  
15 Lubricating oil of low viscosity - 3 pints.

As another specific instance, where a pulpous base is employed which is the waste residue, or oil filtration cakes, from mineral 20 oil purification systems as hereinbefore mentioned, the cakes themselves are fairly impregnated with absorbed oil, so that only about one-third of the amount of make-up oil will be additionally required, when the 25 proportionate amounts will then be approximately

Crushed filtration cake----- 12 pounds.  
Lubricating oil of low viscosity - 1 pint.

30 Either of the foregoing admixtures will provide a substantially non-acidulous and unwatered plastic composition of an immobile or salve-like consistency, which product has a mildly greasy property and yet is 35 slightly viscous to insure a sufficiently tenacious adherence to the greased parts, whereby squeaking or grating noises are eliminated but without interfering with the effectual binding action, essential to frictionally coöperating braking elements.

40 It is also highly desirable, as a commercial expedient especially, that the composition has a pleasing odor, which is satisfactorily accomplished by suitably mixing in an appropriate quantity of a scenting agent 45 as desired, such for instance as oil of mirbane or the like, and the proportionate amount of this scenting agent, for each of the above admixtures, would be approximately twenty centiliters.

50 In such a condition, the admixture is ready for packaging in cans or other suitable receptacles in large or small quantities, but where it is to be marketed in collapsible dispensing tubes especially, it is preferable to also introduce into the admixed composition a suitable thinning agent, such as gasolene or naphtha or other 55 highly volatile cutting liquid, just sufficiently proportionate to give the substance a shade more of plasticity, to enable its being more facilely squeezed out of the usual dispensing tip of the tube, in ribbon form or as otherwise desired, and which volatile 60 thinning agent is promptly evaporated off

upon exposure of the greasing compound for application uses.

In all of the foregoing examples, the amount of the highly volatile thinning agent employed, when the composition is 70 prepared for packaging in collapsible dispensing tubes, would be approximately three pints, so that the admixture of the several ingredients, in the most specific instance set forth, may be indicated in approximately the following proportions:—

Crushed filtration cake----- 12 pounds.  
Lubricating oil of low viscosity ----- 1 pint. 80  
Highly volatile thinning agent, such as gasolene, or the like ----- 3 pints.  
Scenting agent, such as oil of mirbane or the like----- 20 centiliters. 85

While I have thus particularly disclosed my invention, it will nevertheless be understood that I do not restrict myself necessarily to the exact proportions as stated in any of the specific instances, and also that 90 the ingredients may be compounded in much larger and even smaller proportionate quantities than those set forth.

What I do claim, as new and patentable, is:—

1. An anti-squeak composition of matter, compounded from an oil absorptive insoluble earthy base, so proportionately combined and thoroughly admixed with a comparatively small quantity of mineral lubricating 100 oil of low viscosity as to provide an unctuous compound of pasty consistency, substantially as described.

2. An anti-squeak composition of matter, compounded from a major suitable base of 105 infusorial earthy substance, so proportionately combined and thoroughly admixed with a comparatively minimum quantity of lubricating oil of low viscosity as to provide an unctuous compound of pasty consistency, substantially as described. 110

3. An anti-squeak composition of matter, compounded from a major suitable base, substantially consisting of kieselguhr, so proportionately combined and thoroughly 115 admixed with a comparatively minimum quantity of mineral lubricating oil of low viscosity as to provide an unctuous compound of pasty consistency, substantially as described.

4. An anti-squeak composition of matter, compounded from a major suitable base, substantially consisting of an oil absorptive insoluble earthy substance, so proportionately combined and thoroughly admixed 120 with a comparatively minimum quantity of lubricating oil of low viscosity as to provide an unctuous compound of pasty consistency, and the further addition of a highly volatile thinning agent, for cutting 125

130

down the consistency of the paste to a state of quaky plasticity, for packaging purposes, substantially as described.

5. An anti-squeak composition of matter, compounded from a major spongy base, consisting of a ground-up mass of oil filtration cakes, which latter are the waste residue from mineral oil purification systems as hereinbefore disclosed, so proportionately 10 combined and thoroughly admixed with a comparatively minimum quantity of added mineral lubricating oil of low viscosity as to provide an unctuous compound of pasty consistency, substantially as described.
- 15 6. An anti-squeak composition of matter, compounded from the following constituents in the comparatively approximate proportions of twelve pounds of an oil absorp-

tive insoluble base, three pints of lubricating oil of low viscosity, and three pints of 20 a highly volatile thinning agent, all thoroughly admixed, substantially as described.

7. An anti-squeak composition of matter of unctuous properties and plastic consistency, compounded from the following constituents in the comparatively approximate proportions of twelve pounds of an oil absorptive earthy insoluble base, three pints 25 of lubricating oil of low viscosity, three pints of a highly volatile thinning agent, 30 and twenty centiliters of a suitable scenting agent, all thoroughly admixed, substantially as described.

In testimony whereof, I affix my signature.

HAROLD F. WHEELOCK.